

Feb. 24, 1959

K. B. BOZER ET AL

2,875,100

FINISH FOR CELLULOSIC TEXTILE MATERIALS

Filed Oct. 16, 1957



Fig. 2



Cellulosic artificial  
or synthetic silk yarn  
finished with plastified  
film of coal acids  
compounds.

Fig. 1

INVENTORS.  
Keith B. Bozer  
Robert S. Montgomery  
Wesley L. Archer  
BY Griswold & Surdick  
ATTORNEYS

# United States Patent Office

2,875,100

Patented Feb. 24, 1959

1

2,875,100

## FINISH FOR CELLULOSIC TEXTILE MATERIALS

Keith B. Bozer, Robert S. Montgomery, and Wesley L. Archer, Midland, Mich., assignors to The Dow Chemical Company, Midland, Mich., a corporation of Delaware

Application October 16, 1957, Serial No. 690,528

16 Claims. (Cl. 117—139.5)

This invention relates to the finishing of yarns, threads, cords, strings and the like and related filamentary structures and textile materials that are of artificial or synthetic cellulosic origin in order to facilitate their construction into cloth and fabric. The invention has particular reference to the sizing of warp ends of such cellulosic textile materials for subsequent weaving operations. It also relates to the finished cellulosic yarns and the like that are obtainable through its practice.

The cellulosic textile materials that are contemplated as being adapted for employment in the practice of the present invention include any of the essentially or substantially pure artificially regenerated or reconstituted cellulosic materials such as those that have been obtained, for example, from either the viscose, cuprammonium or analogous processes or modified synthetic cellulosic textile materials such as the conventionally available types of cellulose acetate and other cellulose esters of the fiber-forming variety, including cellulose propionate, cellulose butyrate and the like. The viscose rayon and acetate rayon types of so-called artificial or synthetic silk textile fibers are the most common and widely available varieties of the cellulosic textile materials that may advantageously be utilized in the practice of the present invention.

It would be an advantage to provide an effective and relatively inexpensive means for finishing various cellulosic textile yarns and the like, particularly viscose rayon and acetate rayon yarns and filaments. Such a finish would be especially desirable if it could adequately protect the yarn during the course of its construction and conversion into cloth and fabric without exerting any adverse effect upon its physical or chemical constitution. Its utility would be replete and its desirability greatly enhanced if it were capable of temporary or fugitive application and would not require or involve the utilization of unusual or extraordinary scouring techniques to achieve its complete removal from the cellulosic yarn or fabric constructed therefrom. It would be particularly advantageous to provide such means to size warp ends of cellulosic yarn, particularly warp ends of viscose or acetate rayon, for subsequent weaving operations. A cellulosic yarn finished accordingly would be a most proficuous commodity. The achievement of these desiderations and cognate advantages and benefits are, therefore, amongst the principal objects and purposes of the present invention.

To the realization and beneficial achievement of these and related ends, cellulosic yarn of the indicated varieties, including, in particular, viscose rayon and acetate rayon, may advantageously be finished for its construction into cloth and fabric by the application thereto or deposition thereon of a plastified film of mixed aromatic polycarboxylic acid compounds such as may be obtained from the oxidation of coal which, for convenience, are hereinafter referred to as "coal acids compounds." The coal acids compounds may either be the free coal acids, the water-soluble salts, especially the alkali metal (including lithium, sodium and potassium), magnesium and ammonium salts of the coal acids or mixtures thereof. Ad-

2

vantageously, the finishing film of the coal acids compounds may be plastified by a solvent material for the coal acids compounds that are selected from the described group and the finish application may be accomplished with a solution of the coal acids compounds in such solvent material. Preferably, the film is plastified with water and the coal acids compounds are applied in an aqueous solution in order to finish the cellulosic yarn. It is usually desirable and economically attractive to utilize the free coal acids for finishing cellulosic yarn, although in many instances and for many purposes, particularly where a less acidic finish may be required, the water-soluble coal acids salts may be used suitably. It is usually of greatest advantage to size warp ends of cellulosic yarn preparatory to weaving by application of an aqueous solution or mixture of the free coal acids or their water-soluble salts or mixtures of the free coal acids and their salts to the yarn by means of conventional slashing techniques.

Cellulosic yarn of the so-called artificial or synthetic silk variety that is finished or sized in accordance with the present invention with a plastified film of coal acids compounds (which, as indicated, may be comprised of either the free coal acids, their water-soluble salts or mixtures thereof), is adequately lubricated to minimize friction and has excellent resistance to abrasion upon passage through mechanical yarn handling apparatus. This facilitates its being woven or knit into cloth or fabric without injury or operational difficulty. In addition, the yarn is not harmfully or objectionably influenced by either discoloration or diminishment of physical properties due to the presence of the coal acids sizing finish. Besides this, a coal acids compounds finish comprised of either the free acids or their salts, is not injurious or significantly corrosive to the guides and other yarn contacting surfaces and elements in conventional yarn handling and cloth or fabric manufacturing equipment. Furthermore, cellulosic yarn that is provided with a coal acids finish may be scoured to a clean and finish-free condition by conventional techniques using the ordinarily employed detergent baths and scouring agents. The cellulosic yarn that is finished according to the invention is at least commensurate and may frequently be superior in these and other particulars to yarns finished or sized with conventional materials, such as the sodium salts of copolymers of styrene and maleic acid in about equimolar proportions in the polymer molecule, and the like, similar to or identical with that which is available from the Monsanto Chemical Company under the trade-designation "Stymer S." A specimen of an artificial silk cellulosic textile yarn finished in accordance with the present invention is schematically represented in Figure 1 of the accompanying drawing.

Any solvent substance for the coal acids compounds that is inert and non-deleterious to the cellulosic material in the yarn being sized may be employed for formulation of the applying solution and to plastify the finishing substance. It is, as indicated, usually most beneficial and preferred to utilize water for such purpose. However, in many cases, other solvent substances, particularly polar solvents, may be suitable, including glycerine, normally liquid glycols and polyglycols and the like, especially those having relatively high boiling characteristics. Aqueous mixtures of many polar solvents, such as water-glycol combinations, may also be found satisfactory for dissolving and plasticizing the coal acids compounds.

A sufficient quantity of the solvent should be retained in the plastified coal acids compounds film that envelops the yarn as a finish to permit it to be soft, adequately flexible or pliable and sufficiently lubricatory to achieve the desired function. The film should be sufficiently plastified to allow suitable and effective permeation of the yarn, especially when multiple filament yarns are involved,

while remaining in a substantially continuous film phase on the surface of the yarn. It should also be capable of substantially regaining its essential continuity on the surface after having been temporarily broken by such deformations of the yarn as bending or flaring of multiple filament yarns which may occur in handling. Generally, a plastified coal acids compound film that contains between about 0.5 and 10.0 percent by weight of water, based on the weight of the film, will exhibit these desirable properties. A water content in an aqueous plastified coal acids compound film that is in the desired range may usually be simply maintained by keeping the finishing film in equilibrium with air at a relative humidity that is greater than usually normal, as is ordinarily effected in the atmosphere during conventional cloth and fabric manufacturing operations. Such a water content, or equivalent concentrations of other solvents, may usually be achieved in the film after application of the coal acids solution by permitting the applied solution to approach or achieve equilibrium conditions through air drying. In some cases, however, it may be beneficial to employ heat at elevated temperatures in order to more quickly achieve the desired degree of plasticization in the film after application of the solution. As is apparent, the actual water content of aqueous plastified coal acids compounds films is generally dependent on the relative humidity of the atmosphere to which the finish films are exposed.

The cellulosic yarn may be finished so as to pick up or retain any desired quantity of the plastified coal acids compounds film as a finish. For purposes of most fabric construction, there is usually little benefit to be achieved when a finish pick-up greater than about 20 percent by weight, based on the weight of the yarn is exceeded. Advantageously, the pick-up may be between about 0.5 and 10 percent by weight. Oftentimes an amount of the plastified coal acids compounds film on the yarn that is in the neighborhood of 3 percent by weight may be found suitable, especially for purposes of finishing continuous filament yarns. When yarns that have been mechanically spun from staple lengths are being finished, it may sometimes be advantageous to apply comparatively greater quantities of the coal acids compounds film than may be best suited for filament yarns. In addition, especially when spun yarns are being finished, it may also be beneficial to employ thickening agents in the applying solution of the coal acids compounds in order to facilitate achievement of the desired finish pick-up on the yarn.

The finish application may be accomplished readily by immersing the yarn in the aqueous or other solution of coal acids compounds until the desired quantity of the coal acids compounds that are to remain in the plastified finishing film has been assimilated by the yarn. The usual type of operation that is involved in conventional slashing procedures using ordinary slashing or sizing mechanisms may be employed with expedience for such purposes. If desired, however, the aqueous or other solution of the coal acids compounds may be applied to the cellulosic yarn according to other known procedures for the application of textile finishes. Thus, as will be evident to those skilled in the art, roller or wick finish applicators and liquid jet or spray devices and techniques may also be employed for application of the coal acids solution. As mentioned, air or other types of drying, as with the assistance of heated ovens or their equivalent, such as heat lamps, after application of the solution is usually sufficient for formation of the desired film finish. Any cellulosic yarn in twisted or untwisted condition that consists of multiple or individual continuous filament lengths or is fabricated by being spun from staple lengths may advantageously be finished according to the invention.

The mixed aromatic coal acids compounds that are employed for finishing cellulosic yarn in the practice of the invention may be identical with or similar to those which may be obtained by the oxidation with gaseous oxygen, which may be contained in the air, of an aqueous

alkaline slurry of a finely divided carbonaceous material selected from the group consisting of coal and coke that has been obtained by the carbonization of coal at temperatures beneath about 1300° F. Coal acids compounds that have been obtained by the nitric acid oxidation of suitable carbonaceous materials are also generally satisfactory. Such coals that are of the varieties known as anthracite, bituminous and lignite and other low grade coals are generally suitable for production of coal acids. Satisfactory cokes are those produced according to conventional techniques from coal at a temperature beneath about 1300° F. The utilization of higher coking temperatures frequently causes the cokes that are obtained to be graphitic and rendered unsuitable for conversion to coal acids compounds in satisfactory yields.

The preparation of coal acids compounds from coal may, by way of illustration, involve mixing a ground bituminous coal with a caustic alkali, such as sodium hydroxide, and water using an excess of the caustic with respect to the amount that is contemplated as being required for neutralizing the coal acids compounds that are formed. Generally, an apparatus is employed that is constructed from a corrosion-resisting material of construction and that is adapted for operation under pressure. The apparatus is also equipped with an efficient mixing or agitating mechanism and with suitable heat-exchanging means. The weight ratio of the charged ingredients may, for example, be in the proportion of about three parts by weight of the coal to nine parts by weight of the caustic alkali to about one-hundred-twenty-five parts by weight of water. Oxygen is bubbled through the agitated charged ingredients while they are maintained at a temperature between about 390 and 575° F. and under a pressure of from about 500 to 1200 pounds per square inch. The exothermic reaction is continued until substantially all of the carbonaceous ingredients of the coal have gone into solution. This usually requires a period of time between about two and three hours. In the oxidation reaction that occurs, about half of the carbon in the coal is converted to organic acid compounds while the remainder is oxidized to carbon dioxide. Upon termination of the reaction and cooling of the reaction mass, the coal ash is filtered out of the alkali-neutralized coal acids solution that is obtained.

The free coal acids may then be isolated by acidifying the solution with sulfuric acid and, after filtration, recovering the water-soluble free acids by extraction with a suitable water-immiscible solvent, such as methyl ethyl ketone, which does not dissolve in water in the presence of such salts as sodium sulfate, which is obtained in the acidified free coal acids solution. Evaporation and drying techniques may be employed for subsequently isolating the free coal acids. The coal acids may thus be prepared as solid materials that are often pulverized for subsequent handling in a powder form.

The free coal acids products is a hygroscopic, usually yellowish, essentially water soluble material. Its water-soluble salts usually have similar characteristics. The free coal acids product is believed to be substantially comprised of various aromatic polycarboxylic acids. The average molecular weight of the coal acids that are ordinarily obtained is frequently in the neighborhood of 250-270. Their average molecular weight is seldom less than 200 or more than 300. The average equivalent weight of the coal acids is generally about 80; seldom being less than 70 or more than 90. The free coal acids ordinarily appear to have an average of from two and one-half to five carboxylic groups per molecule with an apparent average of about three to four being common. While their exact chemical nature and constitution may be somewhat conjectural, they evidently contain considerable quantities of tri- and tetra-carboxylic benzene acids as well as aromatic acids having more complex nuclei. Frequently, for example, the

greatly preponderant proportion of aromatic nuclei obtained in coal acids compounds prepared in the described fashion have been found to consist of methyl naphthalene, benzene, biphenyl, naphthalene, phenanthrene, alkyl benzene (including toluene) and benzophenone nuclei.

The employment of either the free coal acids, or their water-soluble salts, or mixtures thereof, for finishing cellulosic yarn depends to a great extent, as has been mentioned, on the degree of acidity that is desired in the finish. It is frequently more beneficial and may often be preferred, as indicated, to employ the free coal acids, which generally have a pH near 2, for this purpose. Less acidic finishes of coal acids compounds may be provided by utilization of the salts or various mixtures of the salts (including partial or acid coal acid salts) with the free coal acids product.

By way of further illustration, the efficacy of a coal acids finish on cellulose acetate rayon multiple filament yarn was determined in a series of tests in which a 150 denier, 40 filament nominally twisted yarn was employed. A mixed aromatic free coal acids product was utilized that had been prepared by the alkaline oxidation of coal. The coal acids product had an average molecular weight of about 284 (as determined by boiling point elevation tests), an apparent equivalent weight of about 84.6 and, upon analysis, was found to contain about 54.36 percent by weight of combined carbon, about 3.10 percent by weight of combined hydrogen; about 0.52 percent by weight of combined nitrogen; about 0.16 percent by weight of combined sulfur; and to have a carbon-to-hydrogen ratio of about 1.46:1 with an average functionality or number of carboxylic groups per molecule of about 3.36. The coal acids finish was applied on the yarn by conventional slashing techniques using an aqueous solution of the coal acids that contained about 6 percent by weight of dissolved solids. The resulting plastified coal acids finished film was, with respect to its water content, in substantial equilibrium with air at a temperature of about 70° F. that had a relative humidity of about 65 percent. The equilibrium condition was obtained by conditioning the finished yarn for at least 24 hours in an atmosphere of the indicated character subsequent to the slashing operation. For purposes of comparison, the coal acids finished cellulose acetate yarn was tested along with acetate rayon yarn of the same type that was finished with "Stymer S." The "Stymer S" was employed in a conventional manner ac-

plurality of taut ends of the finished yarn samples to the reciprocal abrading action of a pair of oscillating knife edges that were opposed to one another and in contact in about perpendicular relative disposition with both sides of the yarn. The tests were conducted on a modified version of an apparatus that is known as a Duplan Cohesion Tester (for rayon and raw silk) which is manufactured by Geier & Bluhm, Inc., Troy, New York, and were performed in a generally analogous manner to the equipment manufacturer's recommended procedure. The number of oscillations or cycles required to cause failure of the yarn size and fraying of the yarn were observed in each of the tests. The results of the tests are graphically illustrated in Figure 2 of the accompanying drawing in which the "fray" point, as expressed in the number of cycles required for its accomplishment, is plotted against the quantity of finish on the yarn, expressed in percent by weight, based on the weight of the yarn. The coal acids finished yarn is represented by the solid data points in the graph while the data points obtained on the yarn finished with the "Stymer S" are represented by open circles. For convenience in interpretation, an average or mean value line is drawn through the represented data points. As is apparent, the coal acids finish was at least as effective in protecting the yarn from abrasion as was the conventional "Stymer S" finish.

In order to determine the possible degradative effect of the coal acids on the acetate rayon yarn, two skeins 30 of the same yarn as employed in the foregoing were sized with a coal acids finish using the same coal acids in a similar method of application as are set forth above. One of the skeins was provided with an abnormally large amount of the finish application (in the neighborhood of 10-12 percent by weight, based on the weight of the yarn) while the other was provided with an amount of the size in the neighborhood of 5 percent by weight. Two additional skeins of the same acetate rayon yarn were similarly sized with "Stymer S"; one 35 having an abnormally heavy application of the finish and the other a lesser quantity of finish in the commercially employed range. All of the skeins were then stored under conditions of constant temperature and humidity (about 70° F. and 65 percent relative humidity) for an extended period. The breaking load and percent elongation of each of the sized yarns was determined at frequent intervals during the tests. The results are set forth in the following tabulation.

TABLE 1  
Effect on physical properties of cellulose acetate yarn provided with various sizing finishes

| Time in Days | Breaking Load in Grams                |                                       |                                        |                                        | Percent Elongation |      |      | H-CA         |
|--------------|---------------------------------------|---------------------------------------|----------------------------------------|----------------------------------------|--------------------|------|------|--------------|
|              | (H-S) Heavy Application of "Stymer S" | (L-S) Light Application of "Stymer S" | (L-CA) Light Application of Coal Acids | (H-CA) Heavy Application of Coal Acids | H-S                | L-S  | L-CA |              |
| 6            | 213.2                                 | 161.6                                 | 180.6                                  | 167.4                                  | 7.3                | 8.0  | 18.6 | 13.3         |
| 9            | 183.0                                 | 165.8                                 | 153.4                                  | Average 154.2                          | 7.3                | 20.4 | 14.7 | 10.5         |
| 13           | 183.2                                 | 171.6                                 | 158.8                                  | 164.8                                  | 6.2                | 17.9 | 15.3 | Average 17.0 |
| 16           | 179.2                                 | 165.2                                 | 167.0                                  | 162.8                                  | 5.5                | 17.4 | 19.3 | 11.9         |
| 20           | 163.6                                 | 160.4                                 | 158.5                                  | 164.6                                  | 12.8               | 17.2 | 17.7 | 14.2         |
| 27           | 178.0                                 | 164.6                                 | 175.6                                  | Average 170.4                          | 7.2                | 17.1 | 18.5 | 14.0         |
| 34           | 178.4                                 | 163.2                                 | 162.8                                  | 165.3                                  | 6.0                | 17.5 | 15.1 | Average 17.5 |
| 37           | 174.4                                 | 159.2                                 | 164.2                                  | 155.2                                  | 5.1                | 16.7 | 18.7 | 15.2         |
|              |                                       |                                       |                                        |                                        |                    |      |      | 13.5         |
|              |                                       |                                       |                                        |                                        |                    |      |      | 13.9         |

cording to the manufacturer's recommendation by means of a slasher.

Several samples of both the coal acids finished and the "Stymer S" finished acetate rayon yarn, containing 70 varied amounts of applied finish, were subjected to abrasion tests in which the yarn was run to a "fray" point at which the component individual filaments in the yarn remained flared out or spread apart when the yarn was not under tension. The tests consisted of subjecting a

As is apparent from the foregoing, the coal acids finish exerts little, if any, tendency to degrade the cellulose acetate yarn.

Various scouring tests were performed on the coal acids finished cellulose acetate yarns. In one of the tests, the skein of yarn that had been sized with about 5-6 percent by weight of the water plastified coal acids film was washed with water for about 15 minutes at a temperature between about 100 and 120° F. After the

plain water scouring, the washed yarn was dried and analyzed for residual acid. None could be found. This indicated that the coal acids finish had been completely and readily removed by the plain water wash. In another of the tests, similar yarn samples that have a relatively light coal acids finish applications of about 5-6 percent by weight were examined colorimetrically for traces of finish after having been washed at a temperature of about 150° F. in a 0.25 percent aqueous solution of "Triton X-100," that contained about 0.25 percent by weight of tetradsodium pyrophosphate, and subsequently rinsed for 10 minutes in warm water and dried. "Triton X-100" is an alkylaryl polyester alcohol type of detergent that is available under the indicated trade-designation from Rohm & Haas Company. The samples were compared with a similarly scoured sample of unfinished yarn and also with similar samples that had been finished with the partial sodium salts of the free coal acids which were applied from an applying solution having a pH of about 5 and "Stymer S." The colorimetric examination consisted of wrapping the scoured yarn samples on small white plastic chips and analyzing them with a Model No. 75 Hunter Color and Color-Difference Meter supplied by the Henry A. Gardner Laboratory, Inc. of Bethesda, Maryland. This instrument photometrically measures the amount of reflectance ( $R_d$ ) and color ( $a+b$ ) that is obtainable from the yarn samples. The reflectance value is a measure of the amount of light reflected from the yarn samples in comparison to that reflected from a standard white tile. The color value indicates the deviation of the sample from white. Negative " $a$ " values are indicative of the presence of a blue-green color in the sample and positive " $b$ " values are indicative of the relative degree of yellow that is present. The results that were obtained are included in the following table.

TABLE 2  
Color of various scoured cellulose acetate yarn samples

| Sample                                                     | $R_d$ | $a$  | $b$  |
|------------------------------------------------------------|-------|------|------|
| Unfinished control.....                                    | 88.7  | -1.8 | -0.0 |
| First "Stymer S" finish.....                               | 24.4  | +0.0 | +2.8 |
| Second "Stymer S" finish.....                              | 25.1  | +0.0 | +2.8 |
| First free coal acids finish.....                          | 35.4  | -0.2 | +4.8 |
| Second free coal acids finish.....                         | 34.7  | -0.2 | +4.5 |
| First partial sodium salts of free coal acids finish.....  | 18.0  | -0.8 | +2.9 |
| Second partial sodium salts of free coal acids finish..... | 19.8  | -0.7 | +3.2 |
|                                                            | 20.9  | -0.4 | +2.0 |
|                                                            | 20.7  | -0.4 | +2.0 |
|                                                            | 19.7  | -0.1 | +1.8 |
|                                                            | 19.7  | -0.1 | +1.8 |
|                                                            | 19.9  | -0.3 | +3.8 |
|                                                            | 20.9  | -0.4 | +4.0 |

<sup>1</sup> The increase in yellowness of the sample was believed to be due to some grease which inadvertently became smudged on the yarn while it was being wound on the plastic chip.

<sup>2</sup> This sample was subjected to a great deal more physical handling after the scoured yarn had been wound on the chip than any of the other samples and may have become contaminated with greater soil deposition thereon.

As is evident, the scouring serves to completely remove both the coal acids and their partial sodium salts from the yarn. Had the finishes of the coal acids compounds remained after scouring, the " $b$ " value of the samples finished with the coal acids compounds would have been significantly increased due to the inherent characteristic color of both the free coal acids and their sodium salts.

Excellent results similar to the foregoing may also be obtained when coal acids compounds finishes, including those comprised of other water-soluble coal acids salts such as ammonium or magnesium salts or mixtures thereof with alkali metal salts or with one another or with free coal acids are applied on spun yarns. Excellent results analogous to the foregoing may likewise be obtained when viscose rayon yarns are finished and sized in accordance with the present invention or when cellulosic yarns of the indicated varieties, either filament

or spun, are sized or finished with coal acids compounds for subsequent knitting operations. Furthermore, the coal acids compounds may also be employed with benefit for finishing cellulosic yarns in accordance with the present invention when such compounds are employed in combination with other finishing or sizing materials for yarns of cellulosic origin that are compatible with the coal acids compounds. In addition, samples of filament or other forms of acetate rayon or viscose rayon yarn (for example, acetate yarn similar to that specifically described in the foregoing illustrative specification) that has been sized in accordance with the invention to obtain about 3 percent (or more or less) by weight of the finish film on the yarn may be advantageously employed for both the warp and filling to weave excellent square woven and other fabrics without operational difficulties that might arise if the finish were inadequate for the purpose. Woven coal acids compounds finished fabric is at least as good as similar fabric woven identically from like yarn that is sized with "Stymer S" or other presently employed commercial finishes for the yarn, including starches and oleaginous substances.

What is claimed is:

1. Method for finishing cellulosic yarn selected from the group consisting of regenerated cellulose and fiber-forming cellulose esters to facilitate its construction into cloth and fabric which comprises depositing on the surface of the yarn up to about 20 percent by weight, based on the weight of the yarn, of a plastified film of coal acids compounds selected from the group consisting of free coal acids and mixtures thereof; said coal acids being the water-soluble mixed aromatic polycarboxylic acids that are the products of the oxidation of coal and the like carbonaceous materials, which acids typically have an average molecular weight of from about 200 to 300, an average apparent equivalent weight of from about 70 to 90, and contain an average of from about 2.5 to 5 carboxylic groups per aromatic nucleus in their molecule, said film being plastified with a solvent for said coal acids compounds that is inert to said cellulosic yarn.

2. Method for finishing cellulosic yarn selected from the group consisting of regenerated cellulose and fiber-forming cellulose esters to facilitate its construction into cloth and fabric which comprises applying to the yarn a solution of coal acids compounds selected from the group consisting of free coal acids, water-soluble salts of free coal acids and mixtures thereof, said solution containing a solvent for coal acids compounds that is inert to said cellulosic yarn; and forming therefrom up to about 20 percent by weight, based on the weight of the yarn, of a plastified coal acids film that is plastified with said solvent on the surface of the yarn; said coal acids being the water-soluble mixed aromatic polycarboxylic acids that are the products of the oxidation of coal and the like carbonaceous materials, which acids typically have an average molecular weight of from about 200 to 300, an average apparent equivalent weight of from about 70 to 90, and contain an average of from about 2.5 to 5 carboxylic groups per aromatic nucleus in their molecule.

3. Method for finishing cellulosic yarn selected from the group consisting of regenerated cellulose and fiber-forming cellulose esters to facilitate its construction into cloth and fabric which comprises applying to the yarn an aqueous solution of coal acids compounds selected from the group consisting of free coal acids, water-soluble salts of free coal acids, and mixtures thereof; and forming therefrom up to about 20 percent by weight of a water-plastified coal acids film on the surface of the yarn; said coal acids being the water-soluble mixed aromatic polycarboxylic acids that are the products of the oxidation of coal and the like carbonaceous materials, which acids typically have an average molecular weight of from about 200 to 300, an average apparent equivalent weight of from about 70 to 90, and contain an average of from about 2.5 to 5 carboxylic groups per aromatic nucleus in their molecule.

an average of from about 2.5 to 5 carboxylic groups per aromatic nucleus in their molecule.

4. The method of claim 3, wherein between about 0.5 and 10 percent by weight of said water-plastified film of said coal acids compounds is formed on the surface of the yarn.

5. The method of claim 3, wherein the aqueous applying solution of the coal acids compounds contains between about 0.5 and 30 percent by weight of the coal acids compounds, based on the weight of the solution.

6. The method of claim 3, wherein the aqueous applying solution of the coal acids compounds contains between about 2 and 8 percent by weight of the coal acids compounds, based on the weight of the solution.

7. The method of claim 3 and including the intermediate step of drying the applied aqueous solution of said coal acids compounds to about moisture equilibrium with the surrounding atmosphere to form the plastified film thereof on the surface of the yarn.

8. The method of claim 3, wherein the yarn is a multiple filament yarn.

9. Cellulosic textile yarn selected from the group consisting of regenerated cellulose and fiber-forming cellulose esters provided with up to about 20 percent by weight, based on the weight of the yarn, of a finish comprised of a plastified film of coal acids compounds selected from the group consisting of free coal acids, water-soluble salts of free coal acids, and mixtures thereof; said coal acids being the water-soluble mixed aromatic polycarboxylic acids that are the products of the oxidation of coal and the like carbonaceous materials, which acids typically have an average molecular weight of from about 200 to 300, an average apparent equivalent weight of from about 70 to 90, and contain an average of from about 2.5 to 5 carboxylic groups per aromatic nucleus in their molecule, said film being plastified with a solvent for said coal acids compounds that is inert to said cellulosic yarn.

10. Cellulosic textile yarn selected from the group consisting of regenerated cellulose and fiber-forming cellulose esters provided with up to about 20 percent by weight, based on the weight of the yarn, of a finish comprised of a water plastified film of coal acids compounds selected from the group consisting of free coal acids, water soluble salts of free coal acids, and mixtures thereof; said coal acids being the water-soluble mixed aromatic polycarboxylic acids that are the products of the oxidation of coal and the like carbonaceous materials, which acids typically have an average molecular weight of from about 200 to 300, an average apparent equivalent weight of from about 70 to 90, and contain an average of from about 2.5 to 5 carboxylic groups per aromatic nucleus in their molecule.

11. Cellulosic yarn finished in accordance with claim 10 with between about 0.5 and 10 percent by weight of the water plastified coal acids compound film, based on the weight of the yarn.

12. Cellulosic yarn finished in accordance with claim 10, wherein the water-plastified film of said coal acids compounds is substantially in moisture equilibrium with the surrounding atmosphere.

13. Multiple filament yarn finished according to claim 9.

14. Sized warp ends of yarn in accordance with claim 9.

15. Viscose rayon yarn finished according to claim 9.

16. Cellulose acetate rayon yarn finished according to claim 9.

#### References Cited in the file of this patent

#### UNITED STATES PATENTS

|           |               |               |
|-----------|---------------|---------------|
| 2,199,989 | Dickey et al. | May 7, 1940   |
| 2,292,211 | Dickey        | Aug. 4, 1942  |
| 2,779,684 | Alles         | Jan. 29, 1957 |
| 2,803,607 | Stroh         | Aug. 20, 1957 |
| 2,808,340 | Learn         | Oct. 1, 1957  |